

Patented July 7, 1953

2,644,789

# UNITED STATES PATENT OFFICE

2,644,789

## ELECTRODEPOSITION OF NICKEL

Wilbur J. Shenk, Jr., Shaker Heights, Ohio, assignor to The Harshaw Chemical Company, Cleveland, Ohio, a corporation of Ohio

No Drawing. Application August 2, 1951, Serial No. 240,049

7 Claims. (Cl. 204—49)

1

This invention relates to electrodeposition of metals, and more specifically to a process of, and solutions for use in a process of, electrodepositing nickel, characterized in that the resulting nickel electrodedeposit is bright as it comes from the plating solution. More particularly, the present invention has to do with the discovery of cooperating brightening addition agents suitable for use in an aqueous acid nickel plating solution.

I have now discovered that excellent bright, ductile, and smooth deposits of nickel can be produced over a wide cathode current density range by electrolyzing an aqueous, acid solution of a nickel electrolyte of the class consisting of nickel sulfate, nickel chloride, and mixtures of nickel sulfate with nickel chloride, if such solution also contains an effective amount of each of two cooperating addition agents, one of such addition agents being a bis-pyridinium compound soluble in said solution to the extent of at least .005 gram per liter and characterized in that the two pyridinium groups are connected through a carbon chain or a carbon and oxygen chain, and the other of said addition agents being a cyclic, organic sulfur compound soluble in the acid nickel solution to the extent of at least 0.2 gm. per liter, and selected from the group consisting of organic compounds containing the group



wherein the carbon atom is nuclear carbon, and in which compounds each of the remaining nuclear carbon atoms carries a group of the class consisting of hydrogen, methyl, ethyl, chlorine, bromine, CHO, and phenyl. The first mentioned agent may be referred to as the bis-pyridinium brightener and should be maintained in the plating solution in concentration from 0.005 to 0.05 gram per liter, preferably from 0.001 to 0.005 gram per liter, while the second mentioned addition agent, which I prefer to call a carrier or regulator, should be maintained in the solution in a concentration of from 0.2 to 15.0 gm. per liter, preferably from 1 to 7 gm. per liter.

Since the two above-mentioned classes of addition agents are intrinsically and functionally distinct, they will be separately described and identified.

2

The substances of the first addition agent class, the bis-pyridinium compounds, are soluble in the solution to the extent of at least about .005 gram per liter (for example, in a solution containing 240 grams per liter  $\text{NiSO}_4 \cdot 6\text{H}_2\text{O}$ , 37.5 grams per liter of  $\text{NiCl}_2 \cdot 6\text{H}_2\text{O}$ , and 37.5 grams per liter of  $\text{H}_3\text{BO}_3$ , remainder water), and should be understood to include the unsubstituted pyridinium group and also substituted pyridinium groups such as those having alkyl substituents or substituents coalesced into a ring structure so as to give, for example, isoquinolinium groups.

Addition agents of the first mentioned class are characterized by the presence of two spaced groups of the form,



20 the open valences being satisfied by various substituents such as hydrogen or alkyl (methyl, ethyl, propyl), chlorine, bromine, etc. The general structure may be indicated as follows:



30 where Z may indicate a connecting chain which may be a chain of from 1 to 5 methylene groups or a plurality of chains of from 1 to 5 methylene groups connected through oxygen or phenylene, or a chain of from 1 to 3 phenylene groups, any of the replaceable hydrogens of which may be substituted. The above indicated cyclic nitrogen group, when all the free valences are satisfied by hydrogen, is referred to as a pyridinium group. A plurality of substituents may form a ring structure, for example, isoquinolinium which has the following structure:



45 50 One or more of the hydrogens may be substituted.

## 3

by alkyl giving an alkyl pyridinium group. In general the unsubstituted pyridinium group or the unsubstituted isoquinolinium group is preferred as being simpler, but the substituted groups can be used. The connecting group or chain is made up of methylene and/or phenylene and/or oxygen. It may take the form of a single methylene group, a single phenylene group, or a more complex arrangement. If the pyridinium group, the isoquinolinium group, and substituted pyridinium and isoquinolinium groups are indicated by P and P', the desirable compounds may take such forms as:



10

15

20

These are merely examples, and numerous other arrangements as possible.

To classify these addition agents into sub- 25 classes, most of them fall into three groups, having general formulae as follows:

*Group 1.*—P—[CRR']<sub>n</sub>—O—[CRR']<sub>n'</sub>—O—[CRR']<sub>n'''</sub>—P' where P and P' have the meaning indicated above, R and R' may be, independently, 30 hydrogen, alkyl (methyl, ethyl, propyl), phenyl, etc., n, n' and n''' may be integers from 1 to 5, and n'' may be an integer from 0 to 3.



*Group 2.*—P—[CRR']<sub>n</sub>—P' where P and P' have the meaning indicated above, R and R' may be, independently, hydrogen, alkyl (methyl, ethyl, propyl), phenyl, etc., and n is an integer from 1 to 5.

*Group 3.*—P—[CRR']<sub>n</sub>—(C<sub>6</sub>H<sub>4</sub>—[CRR']<sub>n'</sub>)<sub>n''</sub>—P' where P and P' have the meaning indicated above, R and R' may be, independently, hydrogen, alkyl (methyl, ethyl, propyl), phenyl, etc., n is an integer from 1 to 3, n' is an integer from 0 to 3, and n'' is an integer from 1 to 3.

Some specific examples of the foregoing three groups are as follows:

*Group 1.—Alkylene-ether type linkage*

*a. N,N'-(oxydiethylene)-bis-isoquinolinium chloride*



*b. N,N'-(oxydiethylene)-bis-pyridinium perchlorate*



*c. N,N'-(oxydimethylene)-bis-pyridinium chloride*



*d. N,N'-(oxydimethylene)-bis-isoquinolinium chloride*

The structure is written like (c) but substituting isoquinolinium groups for the pyridinium groups.

*e. N,N'-(oxydimethylene)-bis-(2-methyl-5-ethyl) pyridinium chloride*



*f. N,N'-(oxydi-(trimethylene))-bis-pyridinium chloride*



*g. N,N'-(oxyethylene methylene)-bis-pyridinium chloride*



*h. N,N'-(oxymethylene) isoquinolinium chloride (ethylene) pyridinium chloride*



*i. N,N'-(dioxytriethylene)-bis-pyridinium chloride*



j. *N,N'*-(oxydiethylene)-bis-3-methylisoquinolinium chloridek. *N,N'*-(oxymethylene)-pyridinium chloride-(ethylene)isoquinolinium chloride

## Group 2. Alkylene linkage

a. *N,N'*-ethylene-bis-quinolinium bromideb. *N,N'*-methylene-bis-pyridinium bromidec. *N,N'*-ethylene-bis-pyridinium bromided. *N,N'*-methylene-bis-isoquinolinium bromidee. *N,N'*-methylene-bis-( $\alpha$ -picolinium) bromidef. *N,N'*-cyclohexene-bis-pyridinium bromideg. *N,N'*-styrene-bis-pyridinium bromideh. *N,N'*-methylene-bis-(2-methyl-5-ethylpyridinium) bromide

## Group 3. Alkylene aromatic linkage

a. *N,N'*-(o-xylylene-bis)-pyridinium bromideb. *N,N'*-(p-xylene)-bis-pyridinium bromidec. *N,N'*-(p-xylylene-bis-( $\alpha$ -picolinium)) bromided. *N,N'*-(p-xylylene)-bis-isoquinolinium bromide

Other salts of the foregoing compounds (and others of the same types) may be used with equivalent results, e. g., the chlorides, bromides, acetates, chlorates, etc.

The carriers or regulators constituting the second addition agent class are soluble in the plating solution (for example, in a solution consisting of 240 grams of  $\text{NiSO}_4 \cdot 6\text{H}_2\text{O}$ , 37.5 grams  $\text{NiCl}_2 \cdot 6\text{H}_2\text{O}$ , 37.5 grams of  $\text{H}_3\text{BO}_3$ , and water to make a liter) to the extent of at least 0.2 gram per liter. These 10 include such materials as benzene, naphthalene and thiophene sulfonic acids and salts thereof, and halogen, methyl, ethyl,  $\text{CHO}$ , and phenyl substitution products of the foregoing, such as, for example:

#### CARRIERS OR REGULATORS

1. Benzene mono-sulfonic acid ( $\text{C}_6\text{H}_5\text{SO}_3\text{H}$ )
2. Benzene disulfonic acids ( $\text{C}_6\text{H}_4(\text{SO}_3\text{H})_2$ )
3. Monochlorobenzene monosulfonic acids ( $\text{ClC}_6\text{H}_4\text{SO}_3\text{H}$ )
4. Dichlorobenzene disulfonic acids ( $\text{Cl}_2\text{C}_6\text{H}_2(\text{SO}_3\text{H})_2$ )
5. 2,5-dibromobenzenesulfonic acid ( $\text{Br}_2\text{C}_6\text{H}_3\text{SO}_3\text{H}$ )
6. Toluenesulfonic acids ( $\text{CH}_3\text{C}_6\text{H}_4\text{SO}_3\text{H}$ )
7. Benzaldehydesulfonic acids ( $\text{C}_6\text{H}_4(\text{CHO})\text{SO}_3\text{H}$ )
8. Diphenylsulfonic acids ( $\text{C}_6\text{H}_5\text{C}_6\text{H}_4\text{SO}_3\text{H}$ )
9. Thiophenesulfonic acids ( $\text{C}_4\text{H}_3\text{S}\cdot\text{SO}_3\text{H}$ )
10. Diphenyl sulfone sulfonic acids ( $\text{C}_6\text{H}_5\text{SO}_2\text{C}_6\text{H}_4\text{SO}_3\text{H}$ )
11. Naphthalene disulfonic acids
12. Naphthalene monosulfonic acids
13. Chloronaphthalene disulfonic acids
14. Dibenzenesulfonamide ( $(\text{C}_6\text{H}_5\text{SO}_2)_2\text{NH}$ )
15. Dichloro dibenzenesulfonamides ( $\text{Cl}_2\text{C}_6\text{H}_3\text{SO}_2\text{NHSO}_2\text{C}_6\text{H}_5$ )
16. N-ethane sulfonyl benzene sulfonamide ( $\text{C}_6\text{H}_5\text{SO}_2\text{NHSO}_2\text{C}_2\text{H}_5$ )
17. Potassium, sodium, nickel and cobalt salts of the foregoing
18. Benzene monosulfonamide ( $\text{C}_6\text{H}_4\text{SO}_2\text{NH}_2$ )
19. Saccharine, sodium salt ( $\text{C}_6\text{H}_4\text{SO}_2\text{CONa}$ ) or anhydride ( $\text{C}_6\text{H}_4\text{SO}_2\text{CONH}$ )
20. Benzenesulfonyl chloride ( $\text{C}_6\text{H}_5\text{SO}_2\text{Cl}$ )
21. Chlorobenzenesulfonamides ( $\text{ClC}_6\text{H}_4\text{SO}_2\text{NH}_2$ )
22. Xylenesulfonamides ( $(\text{CH}_3)_2\text{C}_6\text{H}_3\text{SO}_2\text{NH}_2$ )
23. Toluenesulfonamides ( $\text{CH}_3\text{C}_6\text{H}_4\text{SO}_2\text{NH}_2$ )
24. Sulfonated naphthalene. (Mixtures of naphthalene sulfonic acids, produced by treating naphthalene with oleum, preferably two parts of 20% oleum on one part of naphthalene at 160° C. for two hours.)

From these examples it becomes clear that numerous single ring compounds containing the effective group can be used, whether aromatic, such as the benzene sulfonic acids, or heterocyclic with aromatic characteristics, such as thiophene sulfonic acid. Various substituents on the ring structure are exemplified.

It is to be understood that all statements made herein concerning the capabilities of the addition agents presuppose the use of one or a mixture of two or more from each class, i. e., one or a mixture from the bis-pyridinium class and one or a mixture from the class of aromatic sulfur compounds containing the



group. The carrying agents produce a degree of brightness without any brightener, but not enough to yield full brightness alone. I prefer the use of the more common and readily available compounds, and prefer to employ in each addi-

tion agent class only compounds devoid of the group which characterizes the other addition agent class.

The constituents of the bath according to the preferred practice of the invention are (1) water, (2) nickel sulfate, nickel chloride or nickel sulfate with nickel chloride, (3) an aromatic sulfonyl compound such as an aromatic sulfonic acid or a nickel, alkali metal, or cobalt salt thereof, an aromatic sulfonamide, or sulfimide, or a mixture of a plurality thereof, (4) a wetting agent (optional), and (5) a bis-pyridinium compound or a mixture of bis-pyridinium compounds. An additional ingredient of the solution which is desirable is a buffering agent such as boric acid, formic acid, ammonium sulfate, or the like.

It will be noted that in respect to major constituents, the solutions are similar to the well-known "all sulfate," "all chloride," and "sulfate-chloride" or Watts type acid nickel plating solutions. It will be noted also that as to the aromatic sulfonyl type of addition agent or "carrier," as it is often called, the group of suitable materials are of the type which is represented by well-known carriers in the bright nickel plating industry. The essential novel feature of the present invention is the use in such solutions containing the aromatic sulfonyl group of a small amount of a bis-pyridinium compound or a mixture of bis-pyridinium compounds.

The preferred basic solutions in connection with which my invention is realized are as follows:

#### ALL SULFATE

|                                               |                                         |
|-----------------------------------------------|-----------------------------------------|
| 35. $\text{NiSO}_4 \cdot 7\text{H}_2\text{O}$ | 100 to 400 g., preferably 200 to 300 g. |
| Boric acid                                    | 0 to 60 g., preferably 10 to 40 g.      |
| Wetting agent (e. g., sodium lauryl sulfate). | 0 to 0.5 g., preferably 0.05 to 0.2 g.  |
| $\text{H}_2\text{O}$ to make                  | 1000 cc.                                |

#### ALL CHLORIDE

|                                               |                                        |
|-----------------------------------------------|----------------------------------------|
| 50. $\text{NiCl}_2 \cdot 6\text{H}_2\text{O}$ | 50 to 250 g., preferably 100 to 200 g. |
| Boric acid                                    | 0 to 60 g., preferably 10 to 40 g.     |
| Wetting agent (e. g., sodium lauryl sulfate). | 0 to 0.5 g., preferably 0.05 to 0.2 g. |
| $\text{H}_2\text{O}$ to make                  | 1000 cc.                               |

#### SULFATE-CHLORIDE (WATTS TYPE)

|                                               |                                         |
|-----------------------------------------------|-----------------------------------------|
| 55. $\text{NiSO}_4 \cdot 7\text{H}_2\text{O}$ | 100 to 400 g., preferably 200 to 300 g. |
| $\text{NiCl}_2 \cdot 6\text{H}_2\text{O}$     | 10 to 60 g., preferably 25 to 40 g.     |
| Boric acid                                    | 0 to 50 g., preferably 15 to 40 g.      |
| Wetting agent (e. g., sodium lauryl sulfate). | 0 to 0.5 g., preferably 0.025 to 0.2 g. |
| $\text{H}_2\text{O}$ to make                  | 1000 cc.                                |

To each of the foregoing basic solutions I add a suitable quantity of each, or a mixture of two or more of each, of the two co-operating addition agents. One of said addition agents or mixtures is one of the aromatic sulfonyl type, and the other is of the bis-pyridinium type described above. The solution should, for best results, contain an anti-pit agent, although the deposits may be suitable for some purposes without eliminating the pitting, and under some conditions the deposits may not be objectionably pitted even in the absence of an addition agent for control of pitting. Sodium lauryl sulfate or other alkyl sulfate having 8 to 18 carbon atoms may be used as an anti-pit agent, although, as stated, its use is not essential, and other wetting agents or mixtures of wetting agents may be used for control of pitting.

The specific examples in the following table will serve to illustrate the invention, values therein being grams per liter except as otherwise indicated, the balance being water.

|                                                                   | 120   | 300 | 300 | 300 | 300 | 300 | 300 | 300 | 300 | 300 | 300 | 300 | 300 | 300 | 300 | 300 | 300 |
|-------------------------------------------------------------------|-------|-----|-----|-----|-----|-----|-----|-----|-----|-----|-----|-----|-----|-----|-----|-----|-----|
| $\text{NiSO}_4 \cdot 6\text{H}_2\text{O}$                         | 120   | 300 | 300 | 300 | 300 | 300 | 300 | 300 | 300 | 300 | 300 | 300 | 300 | 300 | 300 | 300 | 300 |
| $\text{NiCl}_2 \cdot 7\text{H}_2\text{O}$                         | 120   | 45  | 45  | 45  | 45  | 45  | 45  | 45  | 45  | 45  | 45  | 45  | 45  | 45  | 45  | 45  | 45  |
| $\text{Ni}(\text{BF}_4)_2$                                        |       |     | 35  |     |     |     |     |     |     |     |     |     |     |     |     |     |     |
| $\text{H}_3\text{BO}_3$                                           | 37.5  | 45  | 45  | 45  | 45  | 45  | 45  | 45  | 45  | 45  | 45  | 45  | 45  | 45  | 45  | 45  | 45  |
| Sodium alkyl sulfate (8 to 18 carbon atoms)                       |       |     |     | 0.1 | 0.1 | .25 |     | 0.1 | 0.1 | .25 | 0.1 | 0.1 | 0.1 | 0.1 | 0.1 | 0.1 | 0.1 |
| $\alpha$ -chloro naphthalene disulfonate                          |       |     |     |     |     | 3   |     |     |     |     |     |     |     |     |     |     |     |
| Diphenyl sulfone monosulfonate                                    |       |     |     |     |     |     |     |     |     |     |     |     |     |     |     |     |     |
| Dibenzenesulfonamide                                              | 1     | 1   |     |     | 2.5 | 2.5 |     | 1   | 1   |     | 1   | 1   | 1   | 1   | 1   | 1   | 1   |
| Sulfonated naphthalene, <sup>1</sup> cc. per liter                |       |     |     |     |     |     |     |     |     |     |     |     |     |     |     |     |     |
| 2.5 Dichloro dibenzenesulfonamide                                 |       |     |     |     |     |     |     |     |     |     |     |     |     |     |     |     |     |
| N-carboxy-methyl benzenesulfonamide                               |       |     |     |     |     |     |     |     |     |     |     |     |     |     |     |     |     |
| Benzene monosulfonic acid                                         |       |     |     |     |     |     |     |     |     |     |     |     |     |     |     |     |     |
| Saccharine (Sodium salt)                                          |       |     |     |     |     |     |     |     |     |     |     |     |     |     |     |     |     |
| $\text{N},\text{N}'$ -(dioxytriethylene)-bis-pyridinium chloride  |       |     |     |     |     |     |     |     |     |     |     |     |     |     |     |     |     |
| $\text{N},\text{N}'$ -(oxydiethylene)-bis-isoquinolinium chloride | 0.005 |     |     |     |     |     |     |     |     |     |     |     |     |     |     |     |     |
| $\text{N},\text{N}'$ -methylene-bis-pyridinium bromide            |       |     |     |     |     |     |     |     |     |     |     |     |     |     |     |     |     |
| Para xylene-bis-pyridinium bromide                                | 0.1   |     |     |     |     |     |     |     |     |     |     |     |     |     |     |     |     |
| $\text{N},\text{N}'$ -methylene-bis-isoquinolinium bromide        |       |     |     |     |     |     |     |     |     |     |     |     |     |     |     |     |     |
| $\text{N},\text{N}'$ -cyclohexene-bis-pyridinium bromide          |       |     |     |     |     |     |     |     |     |     |     |     |     |     |     |     |     |
| $\text{N},\text{N}'$ -o-xylene-bis-pyridinium bromide             |       |     |     |     |     |     |     |     |     |     |     |     |     |     |     |     |     |
| Temperature in Degrees Fahrenheit                                 | 140   | 140 | 140 | 140 | 140 | 140 | 140 | 140 | 140 | 140 | 140 | 140 | 140 | 140 | 140 | 140 | 140 |
| Cathode Current Density in Amperes per Square Foot                | 120   | 40  | 100 | 40  | 40  | 40  | 40  | 40  | 40  | 40  | 40  | 40  | 40  | 40  | 40  | 40  | 40  |
| pH                                                                | 3.5   | 4   | 4   | 4   | 4   | 4   | 4   | 4   | 4   | 3.8 | 4   | 4   | 4   | 4   | 4   | 4   | 4   |

<sup>1</sup> Sulfonated naphthalene is the product of reacting 2 parts of 20% oleum on 1 part of naphthalene at 160° C. for 2 hours, neutralizing the resulting mixture with nickel carbonate and diluting to 26° Be. 5 cc. of this product is roughly equal to 1 gram of nickel naphthalene mixed sulfonate.

Having thus described my invention, what I claim is:

1. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness to the deposit, one of said addition agents being a compound comprising two heterocyclic radicals, each containing a nitrogen atom in a 6-membered ring, and said radicals being connected to each other through said nitrogen atoms by means of a carbon-containing group, said group being selected from groups of the class consisting of carbon chains having from 1 to 12 carbon atoms and chains made up of carbon and oxygen and containing not more than a total of 12 connecting atoms between said nitrogen atoms, and the other of said addition agents being an aromatic compound containing the



group, and being soluble in said solution to the extent of at least 0.2 gram per liter, the carbon atom is said



group being nuclear carbon, said first mentioned addition agent being present in concentration from 0.005 to 0.01 gram per liter, and said second mentioned addition agent being present in concentration from 0.2 to 15 grams per liter.

2. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride,

said solution also containing cooperating addition agents capable of imparting brightness to the deposit, one of said addition agents being a compound of the formula,



where  $\text{P}$  and  $\text{P}'$  are radicals of the formula



and the other of said addition agents being an aromatic compound containing the



group, and being soluble in said solution to the extent of at least 0.2 gram per liter, the carbon atom in said



group being nuclear carbon, said first mentioned addition agent being present in concentration from 0.005 to 0.01 gram per liter, and said second mentioned addition agent being present in concentration from 0.2 to 15 grams per liter.

3. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness to the deposit, one of said addition agents being a compound of the formula,



where  $\text{P}$  and  $\text{P}'$  are radicals of the formula

11



and the other of said addition agents being an aromatic compound containing the



group, and being soluble in said solution to the extent of at least 0.2 gram per liter, the carbon atom in said



group being nuclear carbon, said first mentioned addition agent being present in concentration from 0.005 to 0.01 gram per liter, and said second mentioned addition agent being present in concentration from 0.2 to 15 grams per liter.

4. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness to the deposit, one of said addition agents being a compound of the formula,



where P and P' are radicals of the formula



and the other of said addition agents being an aromatic compound containing the



group, and being soluble in said solution to the extent of at least 0.2 gram per liter, the carbon atom in said



group being nuclear carbon, said first mentioned addition agent being present in concentration from 0.005 to 0.01 gram per liter, and said second mentioned addition agent being present in concentration from 0.2 to 15 grams per liter.

5. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness to the

12

deposit, one of said addition agents being a compound of the class consisting of

N,N'-(oxydiethylene)-bis-isoquinolinium salts,  
N,N'-(oxydiethylene)-bis-pyridinium salts,  
N,N'-(oxydimethylene)-bis-pyridinium salts,  
N,N'-(oxydimethylene)-bis-isoquinolinium salts,  
N,N'-(oxydimethylene)-bis-(2-methyl-5-ethyl) pyridinium salts,

10 N,N'-(oxydi(trimethylene))-bis-pyridinium salts,  
N,N'-(oxyethylene-methylene)-bis-pyridinium salts,

N,N'-(oxymethylene)-isoquinolinium (ethylene) pyridinium salts,

N,N'-(dioxytriethylene)-bis-pyridinium salts,  
N,N'-(oxydiethylene)-bis-3-methylisoquinolinium salts,

N,N'-(oxymethylene)-pyridinium(ethylene) isoquinolinium salts,

N,N'-(ethylene)-bis-quinolinium salts,

20 N,N'-(methylene)-bis-pyridinium salts,

N,N'-(ethylene)-bis-pyridinium salts,

N,N'-(methylene)-bis-isoquinolinium salts,

N,N'-(methylene)-bis-( $\alpha$ -picolinium) salts,

25 N,N'-(cyclohexene)-bis-pyridinium salts,

N,N'-(styrene)-bis-pyridinium salts,

N,N'-(methylene)-bis-(2-methyl-5-ethyl) pyridinium salts,

N,N'-(o-xylylene)-bis-pyridinium salts,

30 N,N'-(p-xylylene)-bis-pyridinium salts,

N,N'-(p-xylylene)-bis-( $\alpha$ -picolinium) salts,

N,N'-(p-xylylene)-bis-isoquinolinium salts,

and the other of said addition agents being a cyclic organic compound of the class consisting of

35 Benzene monosulfonic acid,

Benzene disulfonic acids,

Monochlorobenzene monosulfonic acids,

Dichlorobenzene disulfonic acids,

2,5-Dibromobenzenesulfonic acid,

Toluenesulfonic acids,

Benzaldehydesulfonic acids,

Diphenylsulfonic acids,

Thiophenesulfonic acids,

45 Diphenyl sulfone sulfonic acids,

Naphthalene disulfonic acids,

Naphthalene monosulfonic acids,

Chloronaphthalene disulfonic acids,

Dibenzenesulfonamide,

Dichloro dibenzenesulfonamides,

n-Ethane sulfonyl benzene sulfonamide,

Potassium, sodium, nickel and cobalt salts of the foregoing,

Benzene monosulfonamide,

Saccharine, sodium salt or anhydride,

Benzenesulfonyl chloride,

Chlorobenzenesulfonamides,

Xylenesulfonamides,

Toluenesulfonamides,

Sulfonated naphthalene,

60 said first mentioned addition agent being present in concentration from 0.005 to 0.01 gram per liter,

and said second mentioned addition agent being present in concentration from 0.2 to 15 grams per liter.

65 6. A method of electrodepositing nickel in the form of a deposit which is bright as taken from the plating solution without further treatment and which comprises electrolyzing an aqueous, acid solution of a nickel electrolyte of the class consisting of nickel sulfate, nickel chloride, and mixtures of nickel sulfate with nickel chloride, said solution also containing cooperating addition agents capable of imparting brightness to the deposit, one of said addition agents being oxydi-

**13**

ethylene-bis-isoquinolinium chloride, and the other of said addition agents being sulfonated naphthalene, said first mentioned addition agent being present in concentration from 0.005 to 0.01 gram per liter, and said second mentioned addition agent being present in concentration from 0.2 to 15 grams per liter.

7. The invention as defined in claim 6 further characterized in that there is included as a third addition agent, 2,5-dichloro dibenzenesulfonamide in quantity such that the combined concen-

**14**

trations of the sulfonated naphthalene and 2,5-dichloro dibenzenesulfonamide are within the range from 0.2 to 15 grams per liter.

WILBUR J. SHENK, JR.

## 5 References Cited in the file of this patent

## UNITED STATES PATENTS

| Number       | Name  | Date          |
|--------------|-------|---------------|
| 10 2,513,280 | Brown | July 4, 1950  |
| 2,550,449    | Brown | Apr. 24, 1951 |